

Aug. 21, 1945.

C. A. CADWELL

2,383,040

EXOTHERMIC REACTION CHARGE

Filed Dec. 4, 1943



Fig. 1



Fig. 2



Fig. 3

INVENTOR.  
CHARLES A. CADWELL

BY

Oberlin, Limbach & Day.  
ATTORNEYS

## UNITED STATES PATENT OFFICE

2,383,040

## EXOTHERMIC REACTION CHARGE

Charles A. Cadwell, Cleveland Heights, Ohio, assignor to The Electric Railway Improvement Company, Cleveland, Ohio, a corporation of Ohio

Application December 4, 1943, Serial No. 512,913

10 Claims. (Cl. 75—27)

The present improvements, relating as indicated to exothermic reaction charges, have more particular regard to the composition and method of using materials such as are described in my Patent No. 2,229,045, dated January 21, 1941, whereby highly heated molten metal is produced by exothermic reaction.

In such previous patent the composition disclosed is particularly designed for the production of molten copper to be used as a welding material, e. g. to attach the terminal of a copper bond to a steel rail. In attempting to employ the well known exothermic reaction which occurs when a mixture of finely divided aluminum and copper oxide is ignited, the heat yield is sufficient to volatilize whatever copper might be expected from the reaction, and the invention disclosed in my previous patent has as its object the reduction, or rather the absorption, of such excessive heat energy so as to hold the copper yield to a molten rather than a gaseous form. According to the disclosure of said patent this may be accomplished by including in the reaction mixture sufficient copper as metal (preferably alloyed with the aluminum) to absorb a substantial amount of the heat generated by the reaction. As indicated, a charge composed of reaction material such as the foregoing requires relatively high temperature ignition in order to be set off, and for this purpose an igniting powder is placed on top of the charge, such powder being of such composition that it may be ignited by a match or spark and will then generate sufficient heat in turn to ignite the main charge. Such powder should be inflammable enough to jump from a spark point to a quick spread over the whole surface of the charge. However, it has been found in many cases that instead of the reaction thus starting over the whole surface of the charge, it starts at a point, creates a crater and advances downwardly with other portions of the charge falling or rolling into the crater and reacting tardily. The result of such a reaction will be a tandem stream of molten metal rather than the formation of a single compact body such as is desirable, particularly in a rail bonding operation.

I have now discovered that an exothermic reaction of the character described may be satisfactorily controlled so as to produce a single consolidated body of molten metal by making up a charge in layers the composition of which differ in reactivity. Specifically, by disposing on top of the main body of reaction material a small layer of like material having a higher intensity of reaction and then setting off the latter by

means of a further layer of ignition powder, reaction of the entire charge will be brought about in a much more uniform and satisfactory manner than has heretofore been thought possible.

To the accomplishment of the foregoing and related ends, said invention, then, consists of the means hereinafter fully described and particularly pointed out in the claims, the annexed drawing and the following description setting forth in detail certain means and one mode of carrying out the invention, such disclosed means and mode illustrating, however, but one of various ways in which the principle of the invention may be used.

In said annexed drawing:

Fig. 1 is a sectional view of a rail bonding apparatus showing the manner in which my improved exothermic reaction charge may be employed in attaching the terminal of a rail bond to a rail;

Fig. 2 is a perspective view of a cartridge wherein the charge is disposed for convenient use in connection with such apparatus; and

Fig. 3 is a cross-sectional view of such cartridge indicating the disposition of its contents.

The composition which I prefer to employ for the main body of the charge comprises finely divided copper oxide and aluminum, the latter having sufficient copper alloyed therewith to absorb a substantial amount of the heat generated by the reaction. Additional copper as metal may also be provided by utilizing for the copper oxide so-called mill scale, the individual grains of which will be found red at the center from partially oxidized copper, while the surface may be black, highly oxidized and very conducive to quick ignition and combustion. If, however, the powder has been much tumbled and agitated as in a mechanical mixer, the soft black surfaced grain will become a hard surfaced redder grain plus a quantity of segregated fine black dust. Accordingly the oxide content of the powder may be varied by employing a selected grain size. For example, powder that will pass through a 30 mesh screen will have a considerably larger oxygen content than powder which has been passed through a 14 mesh screen.

As illustrated in the several figures of the drawing, the charge is for convenience made up in the form of a package or cartridge by being placed in a suitable container 1 having a closed bottom 2 and a removable top 3.

In assembling the charge there is first placed in the bottom of such container a small layer 4 of igniting powder. Any well known composition of

such powder may be utilized, a satisfactory one being provided by adding a small proportion of red phosphorus to a mixture of finely divided copper oxide and aluminum or copper aluminum alloy.

Directly upon the layer 4 of ignition powder is placed a second similar small layer 5 of reaction material having the same general composition as the main body 6 which composes the remainder of the charge but modified so as to have a higher intensity of reaction. For example, the composition of such main body may be substantially that described in my aforesaid patent as there constituting the entire reaction mass, such body being adapted to yield molten copper having a sufficiently high temperature to effect the welding of a bond terminal to a rail. Thus such main body of the charge may comprise a mixture of about 40 parts of copper oxide and about 17 parts of aluminum including copper alloyed therewith in amount at least equal to the amount of aluminum.

In counterdistinction to the foregoing, the composition of the layer 5 is such as to produce a substantially higher temperature. To secure this, a convenient procedure is to use as the copper oxide component, copper scale of fine particle size such as will pass a 30 mesh screen. As explained above, such powder will have a low content of metallic copper and a high content of copper oxide. It is also desirable to employ an alloy in which the copper content is lower than that of the alloy used in the main body of the charge, e. g. a 60-40 alloy instead of a 65-35 alloy.

The rail bonding apparatus illustrated in Fig. 1 comprises a combined mold and crucible block 10 in which the crucible or reaction chamber 11 is connected with the mold cavity 12 by means of a sprue 13. Such mold cavity is open on one side and formed to hold the terminal 14 of the rail bond against the head 15 of a rail or other part to which such terminal is to be welded. During the welding operation the mold is resiliently held against the rail head by a clamp arm 16 and interposed spring member 17.

A cup-shaped plug 18 composed of metal which will be melted by the heat of the reaction in the crucible chamber is inserted at the bottom of the latter so as to retain the charge in such chamber until the reaction is complete.

For the purpose of properly placing the charge in the crucible, a hinged cover 19 which normally serves to close the upper end thereof is provided with a central opening 20, aligned with the axis of the crucible chamber, an upwardly and outwardly flaring rim 21 surrounding such opening. The opening 20 is of smaller diameter than the container 1 in which the charge is packaged as above described, so that when such container, following removal of cap 3, is placed in an inverted position within rim 21 as shown in dotted outline in Fig. 1, its contents will be discharged into the crucible chamber and assume the form of a slightly mounded body of which the lower portion is composed of the main body 6 of the charge, on the top of which successive thin layers will be superimposed composed of layers 5 and 4 respectively of the charge. If now such layer 4 be ignited as by a spark, ignition of the layer 5 of high intensity powder will immediately follow and because of the composition of such layer the ignition will extend through the entire layer. The latter acts as a booster for the layer of ignition powder, overcoming the ignition resistance of the main body 6 of reaction material by flooding its entire top surface with a flash of high in-

tensity heat. Any streaky ignition of such main body of reaction material is thus avoided, but on the contrary ignition proceeds uniformly downwardly therethrough across the entire section of the mass. The result is the production of a collected body of molten metal in the bottom of the crucible chamber which, as the plug 18 yields, is discharged through the sprue into the mold as a compact falling body rather than as a flowing stream. It thus becomes possible to control quite exactly the amount of heat applied to the welding operation so as to insure the proper attachment of the bond terminal to the rail head without dissolving iron from the surface of the latter or leaving porosities in the resulting cast head.

Other modes of applying the principle of my invention may be employed instead of the one explained, change being made as regards the means and the step herein disclosed, provided those stated by any of the following claims or their equivalent be employed.

I, therefore, particularly point out and distinctly claim as my invention:

1. A self-propagating exothermic reaction charge comprising two contiguously disposed bodies of material wherein a metallic oxide is intermixed with a metallic element capable upon being heated of reducing such oxide to produce molten metal, the amount of such metallic element in each body being sufficient substantially to reduce such intermixed oxide to metal upon ignition of the charge and one of said bodies being relatively smaller and having a higher intensity of reaction than the other, main body.

2. A self-propagating exothermic reaction charge comprising two contiguously disposed bodies of material wherein a metallic oxide is intermixed with a metallic element capable upon being heated of reducing such oxide to produce molten metal the amount of such metallic element in each body being sufficient substantially to reduce such intermixed oxide to metal upon ignition of the charge, one of said bodies being relatively smaller and having a higher intensity of reaction than the other, main body, and a small body of readily ignitable material contiguous to such smaller body of reaction material.

3. A package of material for use in a self-propagating exothermic reaction comprising an elongated container, a main body of material wherein a metallic oxide is intermixed with a metallic element capable upon being heated of reducing such oxide to produce molten metal, such body of material extending from one end of said container towards the other, and a contiguously located, relatively smaller body of such metallic oxide and intermixed metallic element having a higher intensity of reaction the amount of such metallic element in each body being sufficient substantially to reduce such intermixed oxide to metal upon ignition of the charge.

4. A package of material for use in a self-propagating exothermic reaction comprising an elongated container, a main body of material wherein a metallic oxide is intermixed with a metallic element capable upon being heated of reducing such oxide to produce molten metal, such body of material extending from one end of said container towards the other, a contiguously located, relatively smaller body of such metallic oxide and intermixed metallic element having a higher intensity of reaction the amount of such metallic element in each body being sufficient substantially to reduce such intermixed oxide to metal upon ignition of the charge, and a small

layer of readily ignitable material contiguous to such last-mentioned body, the first-mentioned end of said container being openable for discharge of its contents into a reaction chamber.

5. In a method of controlling a self-propagating exothermic reaction of the character described, the steps which comprise placing in a crucible a main body of material wherein a metallic oxide is intermixed with a metallic element capable upon being heated of reducing such oxide to produce molten metal, disposing on top of such body a layer of such metallic oxide and intermixed metallic element having a higher intensity of reaction the amount of such metallic element in each body being sufficient substantially to reduce such intermixed oxide to metal upon ignition of the charge, and setting off such layer which in turn sets off such main body of reaction material.

6. In a method of controlling a self-propagating exothermic reaction of the character described, the steps which comprise placing in a crucible a main body of material wherein a metallic oxide is intermixed with a metallic element capable upon being heated of reducing such oxide to produce molten metal, disposing on top of such body a relatively small layer of such metallic oxide and intermixed metallic element having a higher intensity of reaction the amount of such metallic element in each body being sufficient substantially to reduce such intermixed oxide to metal upon ignition of the charge, disposing on top of such layer a second relatively small layer of readily ignitable material, and then igniting such last-mentioned layer.

7. An exothermic reaction charge comprising two contiguously disposed bodies of intermixed, finely divided copper oxide and aluminum, the

latter being in amount sufficient substantially to reduce such oxide to metal upon ignition of the charge, one of said bodies being relatively smaller than the other and the copper oxide therein having a higher oxygen content than in such other, larger body.

8. An exothermic reaction charge comprising two contiguously disposed bodies of intermixed, finely divided copper oxide and aluminum, together with copper as metal the aluminum being in amount sufficient substantially to reduce such oxide to metal upon ignition of the charge, one of said bodies being relatively smaller than the other and the proportion of metallic copper therein being lower than in such other, larger body.

9. An exothermic reaction charge comprising two contiguously disposed bodies of intermixed, finely divided copper oxide and aluminum, the latter being in amount sufficient substantially to reduce such oxide to metal upon ignition of the charge, one of said bodies being relatively smaller than the other and the size of the copper oxide particles therein being smaller than the size of such particles in the other, larger body.

10. An exothermic reaction charge comprising two contiguously disposed bodies of intermixed, finely divided copper oxide and aluminum, the latter being in amount sufficient substantially to reduce such oxide to metal upon ignition of the charge and having copper alloyed therewith, one of said bodies being relatively smaller than the other, the size of the copper oxide particles in such smaller body being smaller than the size of such particles in such other, larger body, and the percentage of alloyed copper in such smaller body being likewise lower than in such larger body.

CHARLES A. CADWELL.